# EUROPEAN PATENT SPECIFICATION

(11) **EP 2 789 249 B1**
(45) Date of publication and mention of the grant of the patent: **07.11.2018**
(21) Application number: 12856496.0
(22) Date of filing: 09.11.2012
(51) Int. Cl.: A24D 3/10, A24D 3/14

(54) **CIGARETTE FILTER AND CIGARETTE**
ZIGARETTENFILTER UND ZIGARETTE
FILTRE À CIGARETTE ET CIGARETTE

(30) Priority: 06.12.2011 JP 2011267105
(43) Date of publication of application: 15.10.2014
(73) Proprietor: Japan Tobacco, Inc., Tokyo 105-8422 (JP)
(72) Inventor: CHIDA, Masahiro, Tokyo 130-8603 (JP); MUTO, Hiromichi, Tokyo 130-8603 (JP); ITABASHI, Kenichi, Tokyo 130-8603 (JP); SATO, Yukio, Tokyo 130-8603 (JP); NAKAMATSU, Tsutomu, Tokyo 130-8603 (JP); FUJITA, Noritoshi, Tokyo 130-8603 (JP); SUGAI, Kazunori, Tokyo 130-8603 (JP); MIYAUCHI, Masato, Tokyo 130-8603 (JP); MASUI, Tatsuya, Tokyo 130-8603 (JP)
(74) Representative: Isarpatent
(86) International application number: PCT/JP2012/079108
(87) International publication number: WO 2013/084661

(56) References cited:
- EP-A1- 1 470 761
- EP-A1- 1 972 213
- EP-A1- 2 042 635
- EP-A2- 2 446 758
- WO-A1-03/056947
- WO-A1-03/086117
- WO-A1-2009/116417
- JP-A- H0 847 385
- JP-A- S5 955 180
- JP-A- S6 374 477
- JP-A- S6 374 477
- JP-A- 2005 522 208
- JP-A- 2010 521 962
- JP-A- 2011 177 698
- BAGGETT M S ET AL: "Quantitative determination of semivolatile compounds in cigarette smoke", JOURNAL OF CHROMATOGRAPHY, ELSEVIER SCIENCE PUBLISHERS B.V, NL, vol. 97, no. 1, 9 October 1974 (1974-10-09), pages 79-82, XP026483614, ISSN: 0021-9673, DOI: 10.1016/S0021-9673(01)97589-2 [retrieved on 1974-10-09]

## Description

### Technical Field

The present invention relates to a cigarette filter and a cigarette comprising the same.

### Background Art

Many cigarettes comprise filters to remove various components in cigarette mainstream smoke. As the filter, a filter having a cellulose acetate fiber tow as a filter material is widely used.

The acetate filter is known to have selective filtering characteristics such that the filtration efficiency of semivolatile components is higher than the filtration efficiency of tar in cigarette mainstream smoke. The semivolatile component is a component present in both the particulate and vapor phases of cigarette mainstream smoke, and includes a nitrogen-containing compound, ketones, and phenols. These semivolatile components have an effect on cigarette smoking taste, and thus it may be desired that the components are not significantly removed by the filter.

Patent Document 1 discloses a tobacco smoke filter which is substantially formed of cellulose acetate microfilaments having an average diameter of 20 to 250 µm as a tobacco smoke filter for removing harmful components from tobacco smoke. Patent Document 1 also discloses that the microfilaments are mixed with a normal cellulose acetate fiber tow. However, Patent Document 1 does not teach of the semivolatile components, though it discloses that the filter is excellent in removal efficiency of tar in tobacco smoke.

### Prior Art Document

### Patent Document

Patent Document 1: Jpn. Pat. No. 3939823 EP-A-1972213 describes a cigarette filter comprising a filter plug that includes a filter material containing a cellulose acetate fiber tow and cellulosic particles dispersed in the tow, the particles having a sphere equivalent diameter of 200 to 2000 micrometers and a filter-tipped cigarette comprising a cigarette rod and said cigarette filter attached to the end of the cigarette rod. JP-A-S6374477 describes a cigarette filter comprising a filter plug that includes a filter material containing a cellulose acetate fiber tow, and cellulose particles dispersed in the tow, the particles having a sphere equivalent diameter of 0.1 to 200 micrometers and a filter-tipped cigarette comprising a cigarette rod and the cigarette said filter attached to the end of the cigarette rod.

WO-A-03086117 describes a cigarette filter comprising a filter plug that includes a filter material containing a cellulose acetate fiber tow, and cellulose particles dispersed in the tow, the particles having a sphere equivalent diameter of 200 to 1200 micrometers and a filter-tipped cigarette comprising a cigarette rod and the cigarette said filter attached to the end of the cigarette rod.

### Summary of Invention

### Problem to be solved by the Invention

An object of the present invention is to provide a cigarette filter which does not significantly remove a semivolatile component in cigarette mainstream smoke and a cigarette comprising the same.

### Means for solving the Problem

In order to solve the above problem, according to the first aspect of the present invention, there is provided a cigarette filter comprising a filter plug that includes a filter material containing:
a cellulose acetate fiber tow, and
cellulose triacetate particles dispersed in the tow and having an average acetyl substitution degree of 2.8 to 3.0, wherein the cellulose triacetate particles do not contain any additives and have a BET specific surface area of less than 5 m²/g, and account for 1.5 to 30% by volume of the total volume of the filter plug.

According to the second aspect of the present invention, there is provided a filter-tipped cigarette comprising:
a cigarette rod; and
the cigarette filter of the present invention which is attached to the end of the cigarette rod.

### Effects of the Invention

The cigarette filter of the present invention does not significantly remove the semivolatile component in cigarette mainstream smoke.

### Brief Description of Drawings

FIG. 1 is an enlarged schematic view showing a part of a cigarette comprising a filter according to one embodiment of the present invention.
FIG. 2 shows graphs showing relationships between the draw resistance of the control filter and each of the permeability of tar, nicotine, and typical semivolatile components in mainstream smoke.
FIG. 3 shows graphs showing relationships between the draw resistance of the filter according to the present invention and each of the permeability of tar, nicotine, and typical semivolatile components in mainstream smoke.
FIG. 4 is a graph showing a relationship between the selective filtration coefficient Sₓ and the draw resistance of the filter according to the present invention together with that of the control filter.
FIG. 5 is a graph showing a relationship between a plasticizer (triacetin) to be added to a filter material and the permeability of typical semivolatile components.
FIG. 6 is a graph showing a relationship between the draw resistance of the particle-containing filter and the total outer peripheral surface area of the cellulose acetate fiber.
FIG. 7 is a graph showing a relationship between the total outer peripheral surface area of the cellulose acetate fiber forming a filter plug and the permeability of typical semivolatile components.
FIG. 8A is a graph showing the permeability of typical semivolatile components of the filter which is obtained by adding cellulose triacetate particles to a cellulose acetate fiber having a total outer peripheral surface area of 223 cm² on average.
FIG. 8B is a graph showing the permeability of typical semivolatile components of the filter which is obtained by adding cellulose triacetate particles to a cellulose acetate fiber having a total outer peripheral surface area of 255 cm² on average.
FIG. 8C is a graph showing the permeability of typical semivolatile components of the filter which is obtained by adding cellulose particles to a cellulose acetate fiber having a total outer peripheral surface area of 206 cm² on average.
FIG. 9A is a schematic view showing a structure of the filter containing filtration rate control particles used in Example 7.
FIG. 9B is a schematic view showing a structure of the control filter used in Example 7.
FIG. 10 is a graph showing influences of the addition of an additive to the filtration rate control particles on the permeability of typical semivolatile components of the filter.

### Mode for Carrying Out the Invention

Hereinafter, several embodiments of the present invention will be described in detail.

The cigarette filter of the present invention comprises a filter plug which includes a filter material containing a cellulose acetate fiber tow. Cellulose triacetate particles are dispersed in the cellulose acetate fiber tow. The term "dispersed" used herein generally means that the filtration rate control particles are almost uniformly distributed over the entire inside of the cellulose acetate fiber tow (refer to FIG. 1), and the distribution may be weighted toward the side of a cigarette mouthpiece or the side of a cigarette rod. The cellulose triacetate particles play a role in controlling to reduce the filter-filtration rate of the semivolatile components in cigarette mainstream smoke. In addition to the cellulose triacetate particles, it is described but not claimed *per se* that such filtration rate control particles can also be cellulose particles, or a mixture of cellulose particles and cellulose triacetate particles.

Cellulose triacetate particles have an average acetyl substitution degree of 2.76 to 3.00, preferably an average acetyl substitution degree of 2.8 to 3.0, according to the definition of Japan Chemical Fibers Association. In the present invention, the cellulose triacetate particles have an average acetyl substitution degree of 2.8 to 3.0. The average acetyl substitution degree may be measured in accordance with the titration method: ASTM D871-96. The acetyl substitution degree of the cellulose acetate which is determined by the measuring method shows a normal distribution. Accordingly, it is defined as the "average acetyl substitution degree".

The cellulose acetate fibers may be bound with a plasticizer such as triacetin to form a tow. The cellulose acetate fibers are extended in parallel to one another over the total length of the filter.

The cellulose acetate fibers forming the cellulose acetate fiber tow may be cellulose acetate fibers to be used for normal cigarette filters. The cellulose acetate fibers may have a single fineness of 1.5 to 8 deniers and have a sectional shape, such as a circular shape, an oval shape, a Y-shape, an X-shape or an I-shape. The cellulose acetate fibers may be formed of cellulose acetate having an acetyl substitution degree of 2.4 to 2.5 (diacetate). The total fineness of the cellulose acetate fiber tow may be normally from 15000 to 50000 deniers. The cellulose acetate fiber tow is labeled as 1.9Y44000. This means that the single fineness is 1.9 deniers, the fiber cross section has a Y-shape, and the total fineness is 44000 deniers, as well known by those skilled in the art. In the present specification, the unit of the single fineness "denier" represents a weight of a piece of fiber per 9000 m (g/9000 m), and the unit of the total fineness "denier" represents a weight of all pieces of fiber per 9000 m (g/9000 m).

The cellulose particles hardly adsorb the semivolatile components in cigarette mainstream smoke and hardly adsorb menthol either (refer to Examples 1 and 2 below). Further, the cellulose triacetate particles hardly adsorb the semivolatile components in cigarette mainstream smoke and hardly adsorb menthol either (refer to Examples 1 and 2 below). As described above, the filtration rate control particles hardly adsorb menthol. Therefore, in the case where a cigarette filter of the present invention is applied to a menthol cigarette, there is a low possibility that menthol is significantly adsorbed by the filter after production of the cigarette up to when it is smoked by a smoker, and the menthol content in mainstream smoke is hard to be decreased during smoking of the cigarette.

The filtration rate control particles have a granular shape. The average sphere equivalent diameter of the filtration rate control particles is preferably from 100 to 1000 µm, more preferably greater than 250 µm, from the viewpoints of the hardness and draw resistance of the filter, the filtration performance, and the easiness of production of the filter. When producing a filter containing particles having an average sphere equivalent diameter of 100 to 1000 µm, a normal charcoal filter production machine may be directly used (in that case, needless to say, the filtration rate control particles are used in place of charcoal particles). The average sphere equivalent diameter may be obtained by measuring the particle size distribution using a particle size distribution measurement device and calculating the 50% median size of the sphere equivalent diameter, as described in the following examples. According to the present invention, the BET specific surface area of the filtration rate control particles, i.e. the cellulose triacetate particles, is less than 5 m²/g. The BET specific surface area may be determined according to a well-known BET method.

Generally, filtration rate control particles may be obtained with a compression type granulating machine. Specifically, they may be obtained with the compression type granulating machine in the following manner. First, the material of cellulose particles or cellulose triacetate particles is ground into powder. The resulting ground product and various additives are mixed with a precision mixer. Thereafter, the resulting mixture is compaction-molded using a dry granulator while applying a pressure with a roller, and a molded product (e.g., a plate-shaped product) is obtained. Subsequently, the molded product is crushed with a dry particle-size selector. At this time, it is roughly crushed at the first stage, and then it may be crushed into a desired particle size at the second stage. The resulting crushed product is passed through a sieving machine to screen granules having a predetermined particle size. As a result, the filtration rate control particles are prepared. Thus, the filtration rate control particles obtained with the compression type granulating machine are excellent in terms of high yield and fewer problems due to the mixing of long fiber during winding of the filter.

Regarding the filtration rate control particles, the cellulose triacetate particles of the present invention may be obtained by grinding cellulose triacetate flakes and classifying them. Alternatively, the cellulose triacetate particles of the present invention may be obtained by granulating cellulose triacetate flakes with a well-known granulating machine such as of a tumbling type, an extrusion type, a fluid-bed type, a stirring type or a compression type. Further, the cellulose particles described but not claimed *per se* are commercially available.

According to the present invention, the cellulose triacetate particles account for 1.5 to 30% by volume of the volume of the filter containing the cellulose triacetate particles. Further, when considering the production of the filter, if the volume ratio of the added particles increases, the production tends to be difficult. Thus, in order to satisfy the results of the filtration rate control and the sensory evaluation without having any effect of the particles on the production of the filter, the cellulose triacetate particles preferably account for 1.5 to 16% by volume of the volume of the filter containing the filtration rate control particles (refer to Examples 3 and 4 below). Such ratio of the cellulose triacetate particles can achieve a draw resistance of 35 mm H₂O to 180 mm H₂O, which is considered to be suitable for the draw resistance of a filter having a circumference of 24.5 mm and a length of 25 mm. A volume V of the filter may be determined by the equation V = πr²L, where r represents a radius of the filter and L represents a length of the filter (in this regard, the thickness of the filter wrapping paper is of a level small enough to be ignored). The addition weight and the apparent density obtained using a mercury porosimeter were used to calculate the volume of the particles.

If the filtration rate control particles of the present invention, i.e. cellulose triacetate particles, are added to the cellulose acetate fiber tow, the hardness of the resulting filter plug increases. Therefore, triacetin as the plasticizer does not need to be added. Even when triacetin is added as the plasticizer, the addition amount of triacetin as the plasticizer may be decreased. For example, when the cellulose triacetate particles are added to the cellulose acetate fiber tow at the above ratio, a sufficient hardness of the filter plug is obtained by adding triacetin in an amount of 3% by weight or less based on the cellulose acetate fiber tow or not adding (refer to Example 1 below). In this regard, the hardness of the filter plug may be expressed as the amount of strain of the filter plug when an indenter having a diameter of 12 mm is pressed against the filter plug under a 300 g loading for 10 seconds. As the amount of strain is smaller, the filter plug is harder.

Besides the addition of the cellulose triacetate particles to the filter, the addition amount of the plasticizer is decreased or the plasticizer is not added to the filter. As a result, the permeability of semivolatile components can be further improved (refer to Example 6 below).

Further, if the cellulose triacetate particles are added to the cellulose acetate fiber tow, the total outer peripheral surface area of the cellulose acetate fiber can be decreased by 10% or more (usually, 30% or less), as compared to the case where the cellulose triacetate particles are not added. As a result, the permeability of semivolatile components is further improved (refer to Examples 4 and 5 below).

Further, if a filter obtained by adding the cellulose triacetate particles to the cellulose acetate fiber tow is used for the cigarette, the smoking flavor can be changed as compared with the case where a filter not containing the cellulose triacetate particles is used for the cigarette (refer to Example 3 below).

In order to obtain a more preferable cigarette smoking flavor, a small amount of an additive may be added to the cellulose triacetate particles. Example 7 below demonstrates that even if an additive contributing to cigarette smoking flavor is added to the cellulose triacetate particles, no influence is given to the selective permeation of the semivolatile components. The additive may be a component for smoking flavor (e.g., a flavorant) or a component having an effect on the smoking flavor (e.g., a humectant, amino acid, polysaccharide or dietary fiber). Both the components are collectively referred to as a "component contributing to smoking flavor". The addition amount of the component contributing to smoking flavor is preferably 10% by weight or less, and more preferably 5% by weight or less, based on the total weight of the particles (the total weight of the filtration rate control particles and the component contributing to smoking flavor). Examples of the component contributing to smoking flavor include the following flavorants, humectants, amino acids, polysaccharides, and dietary fibers.

The flavorants may be synthetic flavorants, natural flavorants, essential oils, and the like. Further, they may be used regardless of lipophilicity or hydrophilicity. Examples of lipophilic flavorants include vanillin, ethyl vanillin, guarlinalool, thymol, methyl salicylate, linalool, eugenol, menthol, clove, anise, cinnamon, bergamot oil, geranium, lemon oil, spearmint, and ginger. Examples of hydrophilic flavorants include glycerin, propylene glycol, ethyl acetate, and isoamyl alcohol.

Examples of humectants include:
polyols including:
   diols [e.g., an alkanediol (e.g., a C₂₋₁₀ alkanediol such as ethylene glycol, propylene glycol, trimethylene glycol, 1,3-butanediol, 1,4-butanediol, 1,5-pentanediol or hexylene glycol, preferably a C₂₋₈ alkanediol, more preferably a C₂₋₆ alkanediol, particularly a C₂₋₄ alkanediol), and polyalkylene glycol (e.g., diethylene glycol, dipropylene glycol, triethylene glycol or tripropylene glycol)],
   triols [e.g., an alkane triol (e.g., a C₃₋₁₀ alkane triol such as glycerin or 1,2,6-hexanetriol, preferably a C₃₋₆ alkane triol, more preferably a C₃₋₄ alkane triol)], and
   polyols having a tetrafunctional or higher functionality [e.g., a polymer of a polyol (e.g., alkane triols) having a trifunctional or higher functionality (e.g., polyglycerol such as diglycerol or triglycerol)]; and
derivatives of these polyols [e.g., dialkylene glycol monoalkyl ether (e.g., methylcarbitol and ethylcarbitol), and (poly)alkylene glycol monoacylate (e.g., ethylene glycol monoacetate)].

Examples of amino acids include amino acids and salts thereof (amino acid salts). The amino acid may be any of a neutral amino acid (monoamino monocarboxylic acid etc.), an acidic amino acid (monoamino dicarboxylic acid etc.), and a basic amino acid (diaminomonocarboxylic acid etc.), or may be a sulfur-containing amino acid. The amino acid may be an α-amino acid, β-amino acid, γ-amino acid, or the like. Particularly, it may be an α-amino acid. The amino acid may be either an optically active form (D-form, L-form, etc.) or a racemate. Further, examples of amino acids include polyamino acids having a low polymerization degree (e.g., a polymerization degree of 2 to 9, preferably a polymerization degree of 2 to 5, more preferably a polymerization degree of 2 to 3). The amino acid may have a substituent or may be an amino acid derivative in which at least a part of the carboxyl group(s) or the amino group(s) is derivatized. For example, at least a part of the carboxyl group(s) in the amino acid may be a derivatized carboxyl group (e.g., an amide group).

Examples of a typical amino acid include:
an aliphatic amino acid [e.g., an aliphatic monoamino carboxylic acid such as glycine, alanine, isoleucine, leucine, valine, threonine, serine, asparagine, aminosuccinic acid, cysteine, methionine, glutamine or glutamic acid (e.g., an amino-C₂₋₂₀-alkane carboxylic acid, preferably an amino-C₂₋₁₂-alkane carboxylic acid, more preferably an amino-C₂₋₈-alkane carboxylic acid), an aliphatic polyaminocarboxylic acid such as lysine, hydroxylysine, arginine or cystine (e.g., a polyamino-C₂₋₂₀-alkane carboxylic acid, preferably a polyamino-C₂₋₁₂-alkane carboxylic acid)];
an aromatic amino acid (e.g., an aryl-C₂₋₂₀-alkane carboxylic acid such as phenylalanine or tyrosine, preferably a C₆₋₁₀-aryl-C₂₋₁₂-alkane carboxylic acid);
a heterocyclic amino acid (e.g., tryptophan, histidine, proline or 4-hydroxyproline); and
a polypeptide obtained by the polymerization of these amino acids at a low polymerization degree (e.g., at a polymerization degree of 9 or less) (e.g., glycyl glycine, glutamyl glycine, glycyl glycyl glycine, and glycyl proline). Further, examples of amino acid salts include a metal salt [e.g., an alkali metal salt (e.g., a sodium salt such as sodium glutamate)], a hydrochloride (e.g., arginine hydrochloride), and a salt of amino acids (e.g., a salt of lysine with glutamic acid).

Other examples of components contributing to smoking flavor include food additives such as xylitol and mannitol; polymers such as lignin; and polysaccharides or dietary fibers such as cellulose, carboxymethyl cellulose, hydroxypropyl methylcellulose, chitin, starch, glycogen, guar gum, glucomannan, sodium alginate, agarose, chitosan, pectin, carrageenan, and xanthan gum.

Further, a dye may be added to the filtration rate control particles. As the dye, for example, a natural dye extracted from gardenia, safflower, turmeric, annatto, red pepper, paprika, red yeast rice, red cabbage, cacao or the like may be added. The dye may be added in an amount of 0.1 to 5% by weight based on the total weight of the particles (total weight of the filtration rate control particles and the dye). Preferably, it may be added in an amount of 1% by weight or less. The filtration rate control particles containing the dye may have various colors depending on the color of the dye. When the dye is added to the filtration rate control particles and a transparent tipping paper is used to produce a filter, the filtration rate control particles (granules) with which the filter is loaded can be confirmed from the outside. It is known that human feelings can be influenced by color. Accordingly, it is expected that a new feeling is provided to the smoking taste of the cigarette by the color of the dye. Further, when the color of the filtration rate control particles is different from that of the filter fiber, as with charcoal filter, it is possible to easily distinguish between the filtration rate control particles and the filter fiber in the quality inspection in manufacturing the filter.

The filter of the present invention may be attached to one end of a cigarette rod singly or in combination with another filter plug. The latter example is shown in FIG. 1.

FIG. 1 is a schematic view of a cigarette 10 comprising the filter according to one embodiment of the present invention. The cigarette 10 comprises a cigarette rod 110 and a filter 120 which is provided at an end in the axial direction of the cigarette rod 110 in such a manner that the end surface of the filter comes in contact with the end surface of the cigarette rod. The cigarette rod 110 includes a tobacco filler 112 such as tobacco shreds wrapped in a cigarette paper 111. The filter 120 comprises a filter plug 121 of the present invention which includes a tow 122 of a lot of cellulose acetate fibers 123 which are disposed along the axial direction of the filter 120 and may be bundled with a plasticizer such as triacetin. Each of the cellulose acetate fibers 123 is extended over the total length of the filter plug 121. The filtration rate control particles 124 are dispersed in the cellulose acetate fiber tow 122. The filter plug 121 is wrapped in a filter wrapping paper 125. The cigarette rod 110 and the filter 120 are connected with a tipping paper 130, similarly to a normal filter-tipped cigarette. A plurality of ventilation holes 131 may be punched in the tipping paper 130 in one or more rows in the circumferential direction of the filter. A so-called acetate plain filter plug 140 of a cellulose acetate fiber tow 142 wrapped in a filter wrapping paper 141 may be attached to the posterior end of the filter 120 including the filtration rate control particles (to the direction of smoke inhalation). In this case, the filter plug 140 is also wrapped in the tipping paper 130.

### Examples

Hereinafter, the present invention will be described with reference to the examples.

### Example 1

### <Preparation of filtration rate control particles>

### 1. Cellulose triacetate particles

Cellulose triacetate flakes (average acetyl substitution degree: 2.86) were purchased from Daicel Chemical Industries, Ltd. The acetyl substitution degree of the cellulose triacetate flakes was measured in accordance with the titration method: ASTM D871-96. Then, the above-mentioned acetyl substitution degree was confirmed. Subsequently, the cellulose triacetate flakes were ground with a coffee mill (MK-52M manufactured by Matsushita Electric Industrial Co., Ltd.). The ground product was classified through a sieve with an electromagnetic sieve shaker (AS200 control, manufactured by Retsch) to obtain particles at mesh intervals of 300 to 710 µm. As for the particle size distribution, the 50% median size of the sphere equivalent diameter was calculated as the average particle size using a digital-image-analysis type particle size distribution meter (manufactured by Retsch, (sold at HORIBA, Ltd.)). Regarding the resulting particles, the average sphere equivalent diameter was 550 µm, the bulk density was 0.54 g/cc, the apparent density obtained by using a mercury porosimeter was 0.71 g/cc, and the BET specific surface area obtained by nitrogen desorption method was 4.6 m²/g.

### 2. Cellulose particles

Cellulose particles described above but not claimed *per se* were cellulose beads obtained by refining and dissolving wood and forming the resulting viscose into a granular and porous form, and those marketed under the trademark of Viscopearl in Rengo Co., Ltd. were used. Regarding the used particles, the average sphere equivalent diameter was 400 µm, the bulk density was 0.20 g/cc, the apparent density obtained by using a mercury porosimeter was 0.34 g/cc, and the BET specific surface area was below the detection limit.

### <Production of filter plug>

The cellulose particles or cellulose triacetate particles were added to an acetate filter containing triacetin in the same manner as a generally known method for producing a charcoal filter. Further, plain acetate filters not containing filtration rate control particles were also produced. As a filter wrapping paper for each filter plug, one having a basis weight of 24.0 ± 1.5 g/m², a thickness of 60 ± 5 µm, and an air permeability of 10,000 ± 1,800 Coresta unit was used. The diameter of each of the filter plugs was 7.7 mm and the length was 120 mm. The draw resistance of each of the filters was measured according to ISO6565: 2002.

The hardness of the resulting filter plugs was measured as the amount of strain of the filter plug when an indenter having a diameter of 12 mm was pressed against the filter plug under 300 g loading for 10 seconds.

The specification and hardness of the resulting filter plugs are shown in Tables 1A to 1C below.

### [Table 1A]

**Table 1A: Filters containing cellulose triacetate particles**

| Filter Nos. | Specification of cellulose acetate fiber tow | Amount of triacetin (% by weight) | Draw resistance per length of 120 mm (mmH₂O) | Addition amount of particles per filter length of 10 mm (mg/10mm) | Filter hardness (mm) |
|---|---|---|---|---|---|
| A-1 | 3.5Y/35000 | 6 | 418 | 35 | 0.71 |
| A-2 | 5.9Y/35000 | 6 | 319 | 35 | 0.54 |
| A-3 | 2.2Y/35000 | 6 | 570 | 35 | 0.82 |
| A-4 | 3.5Y/35000 | 9 | 396 | 35 | 0.63 |
| A-5 | 3.5Y/35000 | 0 | 420 | 35 | 1.2 |
| A-6 | 5.9Y/35000 | 6 | 423 | 70 | 0.42 |

### [Table 1B]

**Table 1B: Filters containing cellulose particles**

| Filter Nos. | Specification of cellulose acetate fiber tow | Amount of triacetin (% by weight) | Draw resistance per length of 120 mm (mmH₂O) | Addition amount of particles per filter length of 10 mm (mg/10mm) | Filter hardness (mm) |
|---|---|---|---|---|---|
| B-1 | 5.9Y/35000 | 6 | 429 | 35 | 0.52 |
| B-2 | 5.5Y/31000 | 6 | 337 | 35 | 0.77 |
| B-3 | 2.2Y/35000 | 6 | 763 | 35 | 0.77 |
| B-4 | 5.9Y/35000 | 9 | 432 | 35 | 0.48 |
| B-5 | 5.9Y/35000 | 0 | 439 | 35 | 0.97 |
| B-6 | 2.5Y/35000 | 6 | 430 | 10 | 0.97 |

### [Table 1C]

**Table 1C: Acetate plain filters**

| Filter Nos. | Specification of cellulose acetate fiber tow | Amount of triacetin (% by weight) | Draw resistance per length of 120 mm (mmH₂O) | Addition amount of particles per filter length of 10 mm (mg/10mm) | Filter hardness (mm) |
|---|---|---|---|---|---|
| AF-1 | 2.2Y/35000 | 0 | 470 | - | 1.6 |
| AF-2 | 5.9Y/35000 | 0 | 197 | - | 1.6 |
| AF-3 | 2.2Y/35000 | 6 | 433 | - | 1.0 |
| AF-4 | 5.5Y/31000 | 6 | 169 | - | 1.1 |

The hardness of the filters (A-1 to A-6) containing cellulose triacetate particles was from 0.42 to 1.2 (mm). The hardness of the filters (B-1 to B-6) containing cellulose particles was from 0.48 to 0.97 (mm). On the other hand, in the acetate plain filters, the hardness of the acetate plain filters (AF-1 and AF-2) not containing triacetin was 1.6 (mm). Therefore, it was found that the hardness of the filters is increased by the inclusion of the particles in the filters containing cellulose particles and the filters containing cellulose triacetate particles. When the addition amount of the particles is increased, the hardness of the filters can be guaranteed regardless of the addition of triacetin.

### <Production of cigarette sample>

The filter of the commercially available filter-tipped cigarette "Mild Seven Aqua Squash Menthol" was removed. The resultant cigarette rod was connected to a filter for evaluation obtained by cutting the above-produced filter plug into various lengths and placing it in a paper tube (outer diameter: 7.7 mm) with an adhesive tape to produce a cigarette sample. The length and draw resistance of each of the cut filters are shown in Tables 2A to 2C below. It took a month to perform the smoking test after the production of the filters.

### [Table 2A]

**Table 2A: Cut filters containing cellulose triacetate particles**

| Filter plug Nos. (before cutting) | Filter length after cutting (mm) | Draw resistance (mmH₂O) | Marks of cigarettes comprising cut filters |
|---|---|---|---|
| A-1 | 20 | 72 | CA-1 |
| A-2 | 20 | 53 | CA-2 |
| A-3 | 20 | 93 | CA-3 |
| A-4 | 20 | 69 | CA-4 |
| A-5 | 20 | 71 | CA-5 |
| A-6 | 20 | 70 | CA-6 |

### [Table 2B]

**Table 2B: Cut filters containing cellulose particles**

| Filter plug Nos. (before cutting) | Filter length after cutting (mm) | Draw resistance (mmH₂O) | Marks of cigarettes comprising cut filters |
|---|---|---|---|
| B-1 | 20 | 72 | CB-1 |
| B-2 | 20 | 56 | CB-2 |
| B-3 | 20 | 129 | CB-3 |
| B-4 | 20 | 73 | CB-4 |
| B-5 | 20 | 75 | CB-5 |
| B-6 | 20 | 71 | CB-6 |

### [Table 2C]

**Table 2C: Cut filters containing acetate plain filters**

| Filter plug Nos. (before cutting) | Filter length after cutting (mm) | Draw resistance (mmH₂O) | Marks of cigarettes comprising cut filters |
|---|---|---|---|
| AF-3 | 10 | 38 | CAF-3-1 |
| AF-3 | 15 | 55 | CAF-3-2 |
| AF-3 | 20 | 69 | CAF-3-3 |
| AF-3 | 30 | 104 | CAF-3-4 |
| AF-3 | 40 | 133 | CAF-3-5 |
| AF-4 | 10 | 14 | CAF-4-1 |
| AF-4 | 15 | 22 | CAF-4-2 |
| AF-4 | 20 | 28 | CAF-4-3 |
| AF-4 | 30 | 38 | CAF-4-4 |
| AF-4 | 40 | 55 | CAF-4-5 |

### <Smoking test>

Ten cigarette samples produced in the above process (ventilation holes were closed with an adhesive tape) were automatically smoked using an automatic smoking machine (RM20D, manufactured by Borgwaldt KC Inc.) under the following conditions: puff volume: 35.0 mL/2 sec, puff duration: 2 sec/puff, puff interval: 1 puff/min. The particulate matter in cigarette smoke was collected with a Cambridge filter (CM-133, manufactured by Borgwaldt KC Inc.). The smoke passed through the Cambridge filter was collected on 10 mL of methanol cooled to 70°C with a coolant of dry ice and isopropanol.

The Cambridge filter having the particulate matter collected, 10 mL of a methanol solution containing the cigarette smoke collected, and 1 mL of an internal standard solution (d-32 pentadecane: 0.05 mg/mL, d-1-ethanol: 150 mL/L, anethole: 2 mL/L, 1,3-butanediol: 4 mL/L) were added to a serum bottle, which was shaken for 30 minutes. After shaking, the supernatant liquid was collected and used as a sample for analysis. The above operation was also performed on the cigarette rod (control cigarette) obtained by removing the filter of the commercially available filter-tipped cigarette "Mild Seven Aqua Squash Menthol".

### <Analysis of tar, nicotine, and semivolatile components>

The sample for analysis was analyzed by gas chromatography-mass spectrometry (GC-MSD). Agilent 7890A (Agilent Technologies Inc.) was used for GC, and Agilent 5975C (Agilent Technologies Inc.) was used for MSD.

The peak area of each component (standardized by the internal standard) in the chromatogram obtained by the analysis was compared to the peak area of each component in the chromatogram regarding the control cigarette. The permeability "1-Eₓ" of each smoke component through each filter was calculated using the following formula. $1 - Ex = 1 - \frac{\left({A}_{x , in} - {A}_{x , out}\right)}{{A}_{x , in}}$

In the above formula, "A_{x,in}" and "A_{x,out}" represent values obtained by standardizing the peak areas of a component "x" in smoke of the control cigarette and each of the filter-tipped cigarette sample, respectively, by the internal standard. "Ex" represents a filtration rate of the component "x".

As for the semivolatile components, 3-furaldehyde, 2-acetylfuran, and furfural were selected as typical semivolatile components. The average permeability of the components was calculated, and the selective filtration performance of the semivolatile components was evaluated.

Regarding the cigarettes CAF-3-1 to CAF-3-5 and CAF-4-1 to CAF-4-5, the draw resistance of each filter is represented on the horizontal axis, and the logarithm values of the permeability of tar, nicotine, and the typical semivolatile components are plotted on the vertical axis. These are shown in FIG. 2. FIG. 2(A) shows the permeability of tar, FIG. 2(B) shows the permeability of nicotine, and FIG. 2(C) shows the permeability of the typical semivolatile components. In FIGS. 2(A) to 2(C), the circles relate to CAF-3-1 to CAF-3-5, and the triangles relate to CAF-4-1 to CAF-4-5.

Regarding the tar (FIG. 2(A)) and the nicotine (FIG. 2(B)), the permeability can be linearly approximated regardless of the kind of the cellulose acetate tow fiber. Regarding the typical semivolatile components (FIG. 2(C)), the permeability has a different slope depending on the kind of the tow fiber (the diameter of the fiber). This shows that the permeability of tar and nicotine is regulated by only the draw resistance of each filter; however, the permeability behavior of the typical semivolatile components varies depending on the kind of the tow. Since the tar and nicotine are basically particulate phase components, the filtration efficiency may be represented as a function of the draw resistance of each filter. On the other hand, the semivolatile components are distributed to both the vapor phase and the particulate phase, and thus the permeability behavior is influenced by filtration of the particulate phase component and absorption of the vapor phase component to the fiber. As a result, it is not regulated by only the draw resistance.

Subsequently, the results of the cigarettes CA-1 to CA-5 and CB-1 to CB-5 are shown in FIG. 3. FIG. 3(A) shows the permeability of tar, FIG. 3(B) shows the permeability of nicotine, and FIG. 3(C) shows the permeability of the typical semivolatile components. In FIGS. 3(A) and 3(B), a line 'a' relates to CAF-3-1 to CAF-3-3 and CAF-4-4 to CAF-4-5, a line 'b' relates to the cigarettes CA-1 to CA-5, and a line 'c' relates to the cigarettes CB-1 to CB-5. In FIG. 3(C), a line 'a' relates to CAF-3-1 to CAF-3-5 and a line 'b' relates to CAF-4-1 to CAF-4-5.

The results shown in FIGS. 3(A) and 3(B) show that the filter containing the cellulose triacetate particles of the present invention or the cellulose particles described above but not claimed *per se* has a high permeability of tar and nicotine as compared to that of the acetate plain filter, in other words, it has a low filtration rate of tar and nicotine. From the results shown in FIG. 3(C), it is found that the filter containing the cellulose triacetate particles of the present invention or the cellulose particles described above but not claimed *per se* has a high permeability of the semivolatile components as compared to the acetate plain filter. That is, the cellulose triacetate particles of the present invention or the cellulose particles described above but not claimed *per se* allow the permeation of the semivolatile components to be significantly improved. On the other hand, the present inventors have demonstrated that the filter containing the cellulose diacetate particles (average acetyl substitution degree: 2.4 to 2.5) has a function in filtrating the semivolatile components and hardly allows the semivolatile components to be permeated as compared to the acetate plain filter.

From the results shown in FIG. 3(A), the filter containing the cellulose triacetate particles of the present invention or the cellulose particles described above but not claimed *per se* has a different filtration rate of tar from that of the acetate plain filter. In order to reveal the filtering characteristics of the semivolatile components in comparison with tar, the selective filtration coefficient Sₓ was calculated by the following formula as an indicator showing the component selectivity in filtration of the typical semivolatile components. ${S}_{x} = \frac{\left(1 - {E}_{TPM}\right)}{\left(1 - {E}_{x}\right)}$

In the above formula, E_{TPM} represents the filtration rate of crude tar (the total particulate matter).

The selective filtration coefficient Sₓ thus calculated was plotted against the filter draw resistance. The results are shown in FIG. 4. In FIG. 4, a line 'a' relates to the cigarettes CAF-4-1 to CAF-4-5, and a line 'b' relates to CAF-3-1 to CAF-3-5. The results shown in FIG. 4 show the following. When comparing the filters having the same single fineness, the selective filtration coefficient of the filter containing the filtration rate control particles of the present invention is decreased as compared to that of the acetate plain filter in any case of filter draw resistance. Even if the filtration rate of tar is taken into consideration, the semivolatile components are permeated selectively.

Subsequently, in order to examine the effect of the plasticizer (triacetin (GTA)) added to the filter material on the permeability of the typical semivolatile components, as for the cigarette CA-1 (triacetin: 6% by weight), the cigarette CA-4 (triacetin: 9% by weight), the cigarette CA-5 (triacetin: 0%), the cigarette CB-1 (triacetin: 6% by weight), the cigarette CB-4 (triacetin: 9% by weight), and the cigarette CB-5 (triacetin: 0%), the selective filtration coefficient Sₓ of the typical semivolatile components was plotted against the draw resistance. The results are shown in FIG. 5. As shown in FIG. 5, if the addition amount of triacetin is small, it acts in the direction where the semivolatile components are permeated. If the addition amount of triacetin is large, it acts in the direction where the semivolatile components are filtrated. The permeability of the typical semivolatile components can also be controlled by the amount of triacetin. This is because the vapor of the semivolatile components is absorbed (adsorbed) into triacetin on the surface of the cellulose acetate fiber. It is considered that if the addition amount of triacetin is decreased, the adsorption amount of the semivolatile components decreases. In the filter containing the filtration rate control particles of the present invention, even if the addition amount of triacetin is decreased, the filter hardness can be guaranteed. Therefore, a filter which allows the semivolatile components to be more selectively permeated can be achieved by decreasing the addition amount of triacetin.

When the above results are summarized, it was found that the filter containing the cellulose triacetate particles of the present invention or the cellulose particles described above but not claimed *per se* is effective in the selective permeation of the semivolatile components in view of the design of the filter and the easiness in production, although the selective permeation of the semivolatile components can also be controlled by the diameter of cellulose acetate fibers forming a tow and the amount of triacetin.

### Example 2

When the filter of the present invention is intended to be used for a menthol tobacco product, if the adsorption of menthol to the filtration rate control particles of the present invention is continued, the amount of menthol in mainstream smoke is decreased. Therefore, the adsorption amount of menthol to the filtration rate control particles of the present invention was examined.

Specifically, an acetate plain filter (cellulose acetate fiber tow: 1.9Y44000, weight: 30 mg, filter length: 5 mm) was attached to an end of a cigarette rod (circumference: 24.9 mm, length: 59 mm) having 640 mg of tobacco shreds containing 0.59% by weight of menthol. A mentholated acetate filter (cellulose acetate fiber tow: 2.5Y35000, weight: 90 mg, filter length: 15 mm) in which a menthol-containing string was threaded through the center of the filter was arranged at a distance of 5 mm from the acetate plain filter. The cavity between both the filters was filled with the filtration rate control particles of the present invention (cellulose particles or cellulose triacetate particles prepared in Example 1). The content of menthol in the mentholated acetate filter was 1.99% by weight. A cigarette whose cavity is filled with cellulose particles as the filtration rate control particles is designated as a cigarette A, while a cigarette whose cavity is filled with cellulose triacetate particles as the filtration rate control particles is designated as a cigarette B.

The cigarettes thus produced were placed in a glass bottle and sealed, followed by storage at 50°C for two weeks. The cigarette samples after the storage were taken out from the glass bottle. Then, the content of menthol in each of tobacco shreds, acetate plain filters, filtration rate control particles, and mentholated acetate filters was quantified. The content of menthol was quantified by performing methanol-extraction of the samples to be measured (tobacco shreds, acetate plain filters, filtration rate control particles or mentholated acetate filters) and analyzing the methanol-extract with a gas chromatograph (6890 series, manufactured by HEWLETT PACKARD). In the preliminary test, it was confirmed that menthol was extracted with methanol.

The content of menthol in each of tobacco shreds, acetate plain filters, filtration rate control particles, and mentholated acetate filters is shown in Table 3 below.

### [Table 3]

**Table 3: Content of menthol (unit: % by weight)**

| | | Tobacco shreds | Acetate plain filter | Filtration rate control particles | Mentholated acetate filters |
|---|---|---|---|---|---|
| Before storage | | 0.59 | 0 | 0 | 1.99 |
| After storage | Cigarette A | 0.56 | 2.03 | Cellulose particles 0.20 | 1.97 |
| | Cigarette B | 0.43 | 2.30 | Cellulose acetate particles 0.22 | 2.23 |

From the results shown in Table 3, it is found that the cellulose triacetate particles of the present invention or the cellulose particles described above but not claimed *per se* hardly adsorb menthol. Therefore, even if the filter containing the cellulose triacetate particles of the present invention or the cellulose particles described above but not claimed *per se* is used for a menthol tobacco product, the undesired adsorption of menthol to the filtration rate control particles is hardly caused, and thus the menthol smoking taste can be sufficiently experienced.

### Example 3

Filter-tipped cigarettes having the structure shown in FIG. 1 were produced. The tipping paper having ventilation holes punched and a filter were removed from the commercially available filter-tipped cigarette "Mild Seven Aqua Squash Menthol 7 Box", and the obtained cigarette rod was used as the cigarette rod 110 (content of menthol in tobacco shreds: 0.55% by weight). Each of the filters A-1 and A-6 shown in Table 1A, the filters B-1 and B-6 shown in Table 1B, and the filter AF-3 shown in Table 1C was cut into a length of 10 mm so that the filter draw resistance is 35 ± 2 mm H₂O so as to almost constantly keep the amounts of tar, nicotine, and menthol in cigarette mainstream smoke, and the obtained filter plugs were used as the filter plug 121. The acetate plain filter 140 (cellulose acetate fiber tow: 5.0Y35000 (containing 6.9% by weight of triacetin); filter length: 17 mm, menthol content: 2.22% by weight) was attached to the rear end of the filter plug 121. The filter plugs 121 and 140 were connected to the cigarette rod using the tipping paper. It took three months to perform the smoking test after the production of the filters. For confirmation, the specification of the filter plug 121 is shown in Table 4 below.

### [Table 4]

**Table 4: Cut filters**

| Filter plug Nos. (before cutting) | Filter length after cutting (mm) | Draw resistance (mmH₂O) | Marks of cigarettes comprising cut filters |
|---|---|---|---|
| A-1 | 10 | 35±2 | CA-1-2 |
| A-6 | 10 | 35±2 | CA-6-2 |
| B-1 | 10 | 35±2 | CB-1-2 |
| B-6 | 10 | 35±2 | CB-6-2 |
| AF-3 | 10 | 35±2 | CAF-3-1-2 |

Among the cigarettes comprising the filters shown in Table 4, five each of the cigarettes (CA-6-2 and CB-1-2) containing a large amount of the cellulose triacetate particles of the present invention or the cellulose particles described above but not claimed *per se* in the filters thereof and five of the control cigarette (CAF-3-1-2) were smoked without closing the ventilation holes under the smoking conditions described in Example 1. The amounts of tar, nicotine, and menthol in mainstream smoke were measured and the puff number was also measured. The measurement results (averages) of the amounts of tar, nicotine, and menthol per cigarette as well as the puff number are shown in Table 5 below.

### [Table 5]

**Table 5: Amounts of tar, nicotine and menthol in mainstream smoke per cigarette, as well as puff number**

| Cigarette | Tar (mg) | Nicotine (mg) | Menthol (mg) | Puff number |
|---|---|---|---|---|
| CAF-3-1-2 | 7.9 | 0.55 | 0.40 | 6.9 |
| CB-1-2 | 8.8 | 0.62 | 0.45 | 6.9 |
| CA-6-2 | 8.9 | 0.64 | 0.45 | 6.9 |

Subsequently, nine evaluation panelists evaluated the smoking taste of the cigarettes. The evaluation panelists felt the difference in smoking taste between the cigarettes CB-1-2 and CB-6-2 and the control cigarette CAF-3-1-2. As for the characteristics of the smoking flavor of the cigarettes CB-1-2 and CB-6-2, they detected menthol strongly and clearly.

They also felt the difference in smoking taste between the cigarettes CA-1-2 and CA-6-2 and the control cigarette CAF-3-1-2. As for the characteristics of the smoking flavor of the cigarettes CA-1-2 and CA-6-2, they detected menthol strongly and clearly. Further, as for the smoking flavor of the cigarettes CA-1-2 and CA-6-2, they sharply detected the smoking flavor, hardly detected a left bitter taste, and detected a strong tobacco-like flavor. After smoking, they lost the taste immediately and hardly had a strong aftertaste.

### Example 4

Acetate plain filter plugs of various draw resistances (filter length: 10 mm; draw resistance: 14 to 58 mm H₂O) and filter plugs containing the filtration rate control particles of the present invention shown in Table 6 below were produced, and the draw resistance thereof was measured. Regarding the cellulose acetate fiber tows in the produced filters, the total of the outer peripheral surface areas of each single fiber (the total outer peripheral surface area) was calculated in the following manner based on the article (Kazuo Maeda "Research on Development of Tobacco Smoke Filter"), Central Research Institute, Japan Tobacco Inc., December 1983, pages 27 to 30) .

### <Total outer peripheral surface area of cellulose acetate>

(1) The circle equivalent diameter of the single fiber is calculated from the following equation. $Circle equivalent diameter = 11.91 \times {\left(single fineness / fiber density\right)}^{1 / 2}$
   In the above equation, the fiber density is 1.32 g/cm³.
(2) Subsequently, the shape coefficient of the cross section of the single fiber is calculated from the following equation. $Shape coefficient = actual fiber outer peripheral length / \left(4 \times π \times actual cross-sectional area\right)$
   In the above equation, the actual fiber outer peripheral length and the actual cross-sectional area are actually measured from a photomicrograph of the cross section of the single fiber.
(3) Subsequently, the outer peripheral length of the single fiber is calculated from the following equation. $Outer peripheral length of single fiber = π \times circle equivalent diameter \times {\left(shape coefficient\right)}^{1 / 2}$
(4) Finally, the total outer peripheral surface area is determined from the following equation. $Total outer peripheral surface area = outer peripheral length of single fiber \times number of single fiber \times fiber length$

In the above equation, the fiber length is calculated by removing the amount of triacetin from the actually measured weight of the acetate tow to obtain a net weight of the acetate tow and dividing the net weight of the acetate tow by a weight obtained by converting the total fineness into a weight per filter length.

### [Table 6]

**Table 6: Specification of filters**

| Filtration rate control particles | Particle size (µm) | Addition amount of particles per length of 10 cm (mg/10cm) | Specification of cellulose acetate fiber tow | Total outer peripheral surface area of cellulose acetate fiber per filter length of 10 cm (cm²/10cm) | Addition amount of triacetin (% by weight) | Filter length (mm) | Fiber length (mm) | Draw resistance (mmH₂O) | percentage of particles to volume of filters (% by volume) |
|---|---|---|---|---|---|---|---|---|---|
| Cellulose particle | 400 | 35 | 5.5Y31000 | 80 | 6 | 10 | 11.5 | 28 | 22.3 |
| | 400 | 35 | 5.9Y35000 | 87 | 6 | 10 | 11.8 | 36 | 22.3 |
| | 400 | 35 | 2.2Y35000 | 123 | 6 | 10 | 11.4 | 65 | 22.3 |
| | 400 | 35 | 5.9Y35000 | 87 | 0 | 10 | 12.2 | 38 | 22.3 |
| | 400 | 25 | 5.9Y35000 | 87 | 6 | 10 | 11.9 | 28 | 15.9 |
| | 400 | 25 | 5.9Y35000 | 87 | 0 | 10 | 12.0 | 28 | 15.9 |
| | 400 | 25 | 5.9Y35000 | 87 | 3 | 10 | 11.9 | 28 | 15.9 |
| | 700 | 25 | 5.9Y35000 | 87 | 6 | 10 | 12.1 | 27 | 15.9 |
| Cellulose acetate particle | 400 | 35 | 5.9Y35000 | 87 | 6 | 10 | 12.8 | 27 | 10.7 |
| | 400 | 35 | 3.5Y35000 | 108 | 6 | 10 | 12.2 | 36 | 10.7 |
| | 400 | 35 | 2.2Y35000 | 124 | 6 | 10 | 11.6 | 46 | 10.7 |
| | 400 | 70 | 5.9Y35000 | 87 | 6 | 10 | 12.3 | 35 | 21.3 |
| | 400 | 35 | 3.5Y35000 | 108 | 0 | 10 | 12.3 | 35 | 10.7 |
| | 400 | 35 | 5.0Y35000 | 92 | 6 | 10 | 12.1 | 26 | 10.7 |
| | 400 | 35 | 5.0Y35000 | 92 | 0 | 10 | 12.1 | 26 | 10.7 |
| | 400 | 35 | 5.0Y35000 | 92 | 3 | 10 | 12.0 | 26 | 10.7 |

The results are shown in Table 6.

Regarding the results shown in Table 6, the draw resistance of each filter is plotted against the total outer peripheral surface area of each cellulose acetate fiber, and the results are shown in FIG. 6. In FIG. 6, the black rhombuses relate to acetate plain filter plugs, the white triangles relate to filter plugs containing cellulose particles described above but not claimed *per se,* and the white squares relate to filter plugs containing cellulose triacetate particles of the present invention. FIG. 6 shows that, in any case of the draw resistance, the filter plugs containing the cellulose triacetate particles of the present invention or the cellulose particles described above but not claimed *per se* have a smaller total outer peripheral surface area of the cellulose acetate fiber as compared to that of the acetate plain filter plugs. In the filter plugs containing the cellulose triacetate particles of the present invention or the cellulose particles described above but not claimed *per se,* a reduction rate of the total outer peripheral surface area of the cellulose acetate fiber is about from 10 to 30%. Therefore, in the case where the cellulose triacetate particles of the present invention or the cellulose particles described above but not claimed *per se* are added, a cellulose acetate fiber tow having a smaller total outer peripheral surface area can be used as compared to the case where the particles are not added, in producing filter plugs having the same draw resistance.

### Example 5

Regarding the cigarettes CA-1 to CA-6, CB-1 to CB-6, CAF-3-1 to CAF-3-5 and CAF-4-1 to CAF4-5 (refer to Tables 2A to 2C), and the cigarettes comprising the filter plugs shown in Tables 7A and 7B below, the total outer peripheral surface area of the cellulose acetate fiber and the permeability and selective permeation coefficient of the typical semivolatile components were calculated. The results are shown in Tables 8A and 8B below.

### [Table 7A]

**Table 7A: Filters containing cellulose particles (average particle size: 700 µm)**

| Filter Nos. | Specification of cellulose acetate fiber tow | Amount of triacetin (% by weight) | Filter length (mm) | Draw resistance (mmH₂O) | Addition amount of particles per filter length of 10 mm (mg/10mm) | Marks of cigarettes comprising corresponding filters |
|---|---|---|---|---|---|---|
| B2-1 | 5.9Y/35000 | 6 | 20 | 72 | 35 | CB2-1 |
| B2-2 | 2.2Y/35000 | 6 | 20 | 117 | 35 | CB2-2 |
| B2-3 | 5.9Y/35000 | 9 | 20 | 71 | 35 | CB2-3 |
| B2-4 | 5.9Y/35000 | 0 | 20 | 74 | 35 | CB2-4 |
| B2-5 | 2.5Y/35000 | 6 | 20 | 70 | 10 | CB2-5 |

### [Table 7B]

**Table 7B: Acetate plain filters**

| Filter plug Nos. (before cutting) | Filter length after cutting (mm) | Draw resistance (mmH₂O) | Marks of cigarettes comprising cut filters |
|---|---|---|---|
| AF-1 | 10 | 40 | CAF-1-1 |
| AF-1 | 15 | 58 | CAF-1-2 |
| AF-1 | 20 | 76 | CAF-1-3 |
| AF-1 | 30 | 112 | CAF-1-4 |
| AF-1 | 40 | 146 | CAF-1-5 |
| AF-2 | 10 | 18 | CAF-2-1 |
| AF-2 | 15 | 26 | CAF-2-2 |
| AF-2 | 20 | 35 | CAF-2-3 |
| AF-2 | 30 | 53 | CAF-2-4 |
| AF-2 | 40 | 68 | CAF-2-5 |

### [Table 8A]

**Table 8A**

| Cigarette | Total outer peripheral surface area of cellulose acetate fiber (cm²) | Permeability of typical semivolatile components | Selective permeation coefficient of typical semivolatile components |
|---|---|---|---|
| CA-1 | 214 | 0.17 | 3.78 |
| CA-2 | 174 | 0.17 | 4.57 |
| CA-3 | 247 | 0.10 | 5.60 |
| CA-4 | 214 | 0.09 | 7.30 |
| CA-5 | 214 | 0.28 | 2.38 |
| CA-6 | 174 | 0.15 | 4.43 |
| CB-1 | 174 | 0.21 | 3.42 |
| CB-2 | 160 | 0.16 | 4.84 |
| CB-3 | 247 | 0.08 | 6.87 |
| CB-4 | 174 | 0.09 | 7.32 |
| CB-5 | 174 | 0.47 | 1.51 |
| CB-6 | 245 | 0.13 | 4.64 |
| CB2-1 | 174 | 0.18 | 3.84 |
| CB2-2 | 247 | 0.13 | 4.08 |
| CB2-3 | 174 | 0.15 | 4.69 |
| CB2-4 | 174 | 0.45 | 1.56 |
| CB2-5 | 245 | 0.17 | 3.63 |

### [Table 8B]

**Table 8B**

| Cigarette | Total outer peripheral surface area of cellulose acetate fiber (cm²) | Permeability of typical semivolatile components | Selective permeation coefficient of typical semivolatile components |
|---|---|---|---|
| CAF-3-1 | 124 | 0.35 | 2.25 |
| CAF-3-2 | 186 | 0.20 | 3.34 |
| CAF-3-3 | 247 | 0.15 | 3.56 |
| CAF-3-4 | 371 | 0.04 | 11.39 |
| CAF-3-5 | 495 | 0.03 | 12.03 |
| CAF-4-1 | 80 | 0.51 | 1.80 |
| CAF-4-2 | 120 | 0.37 | 2.32 |
| CAF-4-3 | 160 | 0.23 | 3.44 |
| CAF-4-4 | 240 | 0.11 | 6.06 |
| CAF-4-5 | 320 | 0.06 | 9.69 |
| CAF-1-1 | 124 | 0.58 | 1.34 |
| CAF-1-2 | 186 | 0.40 | 1.76 |
| CAF-1-3 | 247 | 0.30 | 2.05 |
| CAF-1-4 | 371 | 0.19 | 2.49 |
| CAF-1-5 | 495 | 0.09 | 3.77 |
| CAF-2-1 | 87 | 0.68 | 1.29 |
| CAF-2-2 | 131 | 0.61 | 1.40 |
| CAF-2-3 | 174 | 0.54 | 1.49 |
| CAF-2-4 | 262 | 0.37 | 1.88 |
| CAF-2-5 | 349 | 0.25 | 2.28 |

Regarding the results shown in Tables 8A and 8B, the permeability of the typical semivolatile components is plotted against the total outer peripheral surface area of the cellulose acetate fiber, and the results are shown in FIG. 7. In FIG. 7, the white triangles relate to the cigarettes CB-5 and CB2-4, the white squares relate to the cigarette CA-5, the white circles relate to the cigarettes CAF-1-1 to CAF-1-5, and the white rhombuses relate to the cigarettes CAF-2-1 to CAF-2-5. The plasticizer is not contained in the filter plugs of any of the above-mentioned cigarettes. In FIG. 7, the black triangles relate to the cigarettes CB-1, CB-2, CB-3, CB-6, CB2-1, CB2-2, and CB2-5, the black squares relate to the cigarettes CA-1, CA-2, CA-3, and CA-6, the black circles relate to the cigarettes CAF-3-1 to CAF-3-5, and the black rhombuses relate to the cigarettes CAF-4-1 to CAF-4-5. The plasticizer is contained in the filter plugs of all the above-mentioned cigarettes.

From FIG. 7, it is found that the permeability of the typical semivolatile components in each of the acetate plain filter plugs is largely dependent on the addition amount of the plasticizer (triacetin); however, in the case of the same amount of the plasticizer, the permeability of the typical semivolatile components is determined by the total outer peripheral surface area of the cellulose acetate fiber. Further, it is found that the particle size of cellulose particles described above but not claimed *per* se has no influence on the filtering characteristics of the semivolatile components. These facts are attributed to the fact that cellulose particles described above but not claimed *per se* and cellulose triacetate particles of the present invention are not easily dissolved in an acetone solvent and hardly adsorb menthol or triacetin, and thus they have a low adsorbing ability for semivolatile components having a polarity close to that of menthol or triacetin.

FIG. 7 shows that the selective filtering characteristics of the semivolatile components can be controlled by changing the kind of the cellulose acetate fiber tow or the addition amount of the plasticizer. However, since a certain level of hardness of the filter needs to be guaranteed and the draw resistance needs to be controlled when setting the amounts of tar and nicotine in mainstream smoke, it is not possible to freely combine the kind of the cellulose acetate fiber tow and the addition amount of the plasticizer for cigarette products. However, if the cellulose triacetate particles of the present invention or the cellulose particles described above but not claimed *per se* are added to a filter according to the present invention, the constant hardness of the filter can be maintained by the presence of the particles even if the addition amount of triacetin is decreased, and the draw resistance can be controlled by the addition of the particles in order to adjust the amount of tar/nicotine in mainstream smoke to a desired value. Therefore, the cellulose acetate fiber tow regarded as unusable in the prior art (i.e., a cellulose acetate fiber tow whose total outer peripheral surface area is small) can be used according to the present invention. In other words, generally, as the total outer peripheral surface area of the cellulose acetate fiber becomes smaller, the draw resistance of the filter plug tends to decrease. Thus, a cellulose acetate fiber tow having the draw resistance lower than that of the cellulose acetate fiber tow of the conventional cigarette filter can be used. As a result, it is possible to develop a filter having characteristics in which the semivolatile components are permeated selectively as compared to tar.

As described above, it is found that, if the cellulose triacetate particles of the present invention or the cellulose particles described above but not claimed *per se* are added to a filter according to the present invention, the control width of the permeation of the semivolatile components can be extended, which has been limited in the conventional acetate plain filter in view of product design or production. Thus, the present invention is effective in providing new tobacco smoking flavor or new menthol tobacco smoking flavor.

### Example 6

The cellulose powder (FMC Biopolymer, trade name: Endurance MCC) and the cellulose triacetate powder (Daicel Chemical Industries, Ltd., trade name: Acetate Flake DS2.9 LT-55 (TAC)) were used as raw materials. Each powder was pressurized at 20 Mpa for 10 minutes using a tablet molding machine (manufactured by Jasco Corporation) and a hydraulic hand pump (manufactured by Riken Seiki Co., Ltd.) to obtain a plate-shaped molded product. Subsequently, the resulting plate-shaped molded product was ground with a coffee mill (MK-52M manufactured by Matsushita Electric Industrial Co., Ltd.). The ground product was classified through a sieve with an electromagnetic sieve shaker (AS200 control, manufactured by Retsch) to produce filtration rate control particles at mesh intervals of 300 to 710 µm. The resulting the cellulose triacetate particles of the present invention or the cellulose particles described above but not claimed *per se* were used to produce respectively filters containing cellulose triacetate particles of the present invention and filters containing cellulose particles described above but not claimed *per se* according to the same procedure as Example 1. The draw resistance and hardness of the produced filters were measured according to the same procedure as Example 1.

The specification and hardness of the resulting filter plugs are shown in Tables 9A and 9B below.

### [Table 9A]

**Table 9A: Filters containing cellulose triacetate particles**

| Filter Nos. | Specification of cellulose acetate fiber tow | Addition amount of triacetin (% by weight) | Draw resistance per length of 120 mm (mmH₂O) | Addition amount of particles per filter length of 10 mm (mg/10mm) | Filter hardness (mm) |
|---|---|---|---|---|---|
| A-7 | 5.0Y35000 | 6 | 311 | 35 | 0.54 |
| A-8 | 5.0Y35000 | 3 | 307 | 35 | 0.70 |
| A-9 | 5.0Y35000 | 0 | 314 | 35 | 1.2 |
| A-10 | 3.5Y35000 | 6 | 327 | 29 | 0.75 |
| A-11 | 3.5Y35000 | 3 | 332 | 29 | 1.0 |
| A-12 | 3.5Y35000 | 1 | 322 | 29 | 1.3 |

### [Table 9B]

**Table 9B: Filters containing cellulose particles**

| Filter Nos. | Specification of cellulose acetate fiber tow | Addition amount of triacetin (% by weight) | Draw resistance per length of 120 mm (mmH₂O) | Addition amount of particles per filter length of 10 mm (mg/10mm) | Filter hardness (mm) |
|---|---|---|---|---|---|
| B-7 | 5.9Y35000 | 6 | 339 | 25 | 0.52 |
| B-8 | 5.9Y35000 | 3 | 334 | 25 | 0.7 |
| B-9 | 5.9Y35000 | 0 | 331 | 25 | 1.0 |
| B-10 | 5.0Y35000 | 6 | 343 | 21 | 0.65 |
| B-11 | 5.0Y35000 | 1 | 321 | 21 | 1.1 |

In Tables 9A and 9B, the addition amount of triacetin is expressed in percent by weight based on the cellulose acetate fiber tow.

The hardness of the filters (A-7 to A-12) containing cellulose triacetate particles was from 0.54 to 1.3 (mm). The hardness of the filters (B-7 to B-12) containing cellulose particles was from 0.52 to 1.1 (mm). On the other hand, in the acetate plain filters, the hardness of the acetate plain filters (AF-1 and AF-2) not containing triacetin was 1.6 (mm). Therefore, it was found that the hardness of the filters is increased by the inclusion of the particles in the filters containing cellulose particles described above but not claimed *per se* and the filters containing cellulose triacetate particles of the present invention. When the addition amount of the particles is increased, the hardness of the filters can be guaranteed even if the addition amount of triacetin is decreased. Specifically, it was found that when 3% by weight or less of triacetin was added or even when triacetin was not added, the sufficient hardness of the filter plugs was obtained.

### <Production of cigarette samples>

The filter of commercially available filter-tipped cigarette "Seven Stars Solid Menthol" was removed. The resultant cigarette rod was connected to a filter for evaluation obtained by cutting the above-produced filter plug into various lengths and placing it in a paper tube (outer diameter: 7.7 mm) with an adhesive tape to produce a cigarette sample. It took two months to perform the smoking test after the production of the filters. The length and draw resistance of each of the cut filters as well as the total outer peripheral surface area of the cellulose acetate fiber are shown in Tables 10A and 10B below.

### [Table 10A]

**Table 10A: Cut filters containing cellulose triacetate particles**

| Filter plug Nos. (before cutting) | Filter length after cutting (mm) | Draw resistance (mmH₂O) | Total outer peripheral surface area of cellulose acetate fiber (cm²) | Marks of cigarettes comprising cut filters |
|---|---|---|---|---|
| A-7 | 20 | 54 | 223 | CA-7 |
| A-8 | 20 | 53 | 222 | CA-8 |
| A-9 | 20 | 54 | 224 | CA-9 |
| A-10 | 20 | 53 | 255 | CA-10 |
| A-11 | 20 | 54 | 256 | CA-11 |
| A-12 | 20 | 56 | 255 | CA-12 |

### [Table 10B]

**Table 10B: Cut filters containing cellulose particles**

| Filter plus Nos. (before cutting) | Filter length after cutting (mm) | Draw resistance (mmH₂O) | Total outer peripheral surface area of cellulose acetate fiber (cm²) | Marks of cigarettes comprising cur filters |
|---|---|---|---|---|
| B-7 | 20 | 56 | 202 | CB-7 |
| B-8 | 20 | 57 | 202 | CB-8 |
| B-9 | 20 | 59 | 204 | CB-9 |
| B-10 | 20 | 62 | 207 | CB-10 |
| B-11 | 20 | 58 | 214 | CB-11 |

The produced cigarettes CA-7 to CA-12 and CB-7 to CB-11 were subjected to the smoking test according to the same procedure as Example 1. The smoking test was also performed on the cigarette rod (control cigarette) obtained by removing the filter of the commercially available filter-tipped cigarette "Seven Stars Solid Menthol".

The sample for analysis obtained in the smoking test was used to analyze tar, nicotine, and the semivolatile components according to the same procedure as Example 1. The permeability (%) and the selective filtration coefficient (%) were calculated according to the same numerical formulae described in Example 1.

The permeability and selective filtration coefficient of the typical semivolatile components of the cigarettes CA-7 to CA-12 and CB-7 to CB-11 are shown in Tables 11A to 11C below with respect to each total outer peripheral surface area of the cellulose acetate fiber.

### [Table 11A]

**Table 11A: Permeability and selective filtration coefficient of typical semivolatile components**

| Filter | CA-7 | CA-8 | CA-9 |
|---|---|---|---|
| Permeability (%) | 20 | 28 | 32 |
| Selective permeation coefficient (%) | 316 | 244 | 193 |

### [Table 11B]

**Table 11B: Permeability and selective filtration coefficient of typical semivolatile components**

| Filter | CA-10 | CA-11 | CA-12 |
|---|---|---|---|
| Permeability (%) | 27 | 30 | 35 |
| Selective permeation coefficient (%) | 252 | 220 | 192 |

### [Table 11C]

**Table 11C: Permeability and selective filtration coefficient of typical semivolatile components**

| Filter | CB-7 | CB-8 | CB-9 | CB-10 | CB-11 |
|---|---|---|---|---|---|
| Permeability (%) | 26 | 31 | 44 | 28 | 42 |
| Selective permeation coefficient (%) | 285 | 221 | 159 | 256 | 162 |

The permeability of the typical semivolatile components of the cigarettes CA-7 to CA-12 and CB-7 to CB-11 is shown in FIGS. 8A to 8C with respect to each total outer peripheral surface area of the cellulose acetate fiber.

FIG. 8A shows the permeability of the typical semivolatile components of the filters containing cellulose triacetate particles of the present invention in the case where the total outer peripheral surface area of the cellulose acetate fiber is 223 cm² (the specification of the fiber tow: 5.0Y35000). FIG. 8B shows the permeability of the typical semivolatile components of the filters containing cellulose triacetate particles of the present invention in the case where the total outer peripheral surface area of the cellulose acetate fiber is 255 cm² (the specification of the fiber tow: 3.5Y35000). FIG. 8C shows the permeability of the typical semivolatile components of the filters containing cellulose particles described above but not claimed *per se* in the case where the total outer peripheral surface area of the cellulose acetate fiber is 206 cm² (the specification of the fiber tow: 5.9Y35000 and 5.0Y35000).

From the results of Tables 11A to 11C and FIGS. 8A to 8C, it is confirmed that when the filters having almost the same total outer peripheral surface area of the cellulose acetate fiber are compared to one another, the permeability of the typical semivolatile components is high in the filters having a small addition amount of the plasticizer. This is because the amount of adsorption of the semivolatile components to the surface of the cellulose acetate fiber is increased by the plasticizer. Therefore, the permeation of the semivolatile components can be further improved by decreasing the addition amount of the plasticizer or not adding the plasticizer, in addition to adding the cellulose triacetate particles of the present invention or the cellulose particles described above but not claimed *per se* to a filter.

### Example 7

In order to examine the influences of the additives on the filtration performance of the filtration rate control particles, cellulose particles and the cellulose particles containing the additives described in Table 12 below were prepared. The cellulose particles were prepared by the same procedure as Example 6. The cellulose particles containing the additives were prepared by mixing the additives and cellulose powder according to the same procedure as Example 6. The additives were added in amounts described in Table 12. In Table 12, the "addition amount" is represented by a ratio (% by weight) of the additives to the total weight of the filtration rate control particles and the additives. The filtration rate control particles not containing the additives were also prepared for comparison.

### [Table 12]

**Table 12: Additive-added filtration rate control particles**

| Filtration rate control particle Nos. | Additives | Addition amount (%) |
|---|---|---|
| A-1 | - | - |
| B-1 | L-arginine | 5 |
| B-2 | L-alanine | 5 |
| B-3 | L-glutamic acid | 5 |
| B-4 | Lignin | 10 |
| B-5 | Powder sugar | 2 |
| B-6 | Pectin | 10 |
| B-7 | Sorbitol | 5 |

### <Production of filter plug>

In order to evaluate the filtration performance of the filtration rate control particles, the filtration rate control particles A-1 and B-1 to B-7 were used to produce filter plugs F-A-1 and F-B-1 to F-B-7. As shown in FIG. 9A, the filtration rate control particles were arranged in a paper tube having a length of 25 mm. Acetate filters (5 mm) were placed at the front side (the side of a tobacco rod) and the rear side (the side of a filter mouthpiece) of the filtration rate control particles so as to cover the filtration rate control particles. Thus, filters filled with the filtration rate control particles were produced. The addition amounts of the filtration rate control particles are shown in Table 13. As shown in FIG. 9B, a filter plug F-C-1 having two acetate filters (5 mm) arranged in a paper tube having a length of 25 mm was produced as a control. The specification of each of the filters is shown in Table 13.

### [Table 13]

**Table 13: Specification of filters**

| Filter Nos. | Filtration rate control particle Nos. | Addition amount (mg) | Draw resistance of filter (mmH₂O) | Draw resistance of filtration rate control particles (mmH₂O) |
|---|---|---|---|---|
| F-A-1 | A-1 | 100 | 68 | 54 |
| F-B-1 | B-1 | 100 | 55 | 41 |
| F-B-2 | B-2 | 100 | 53 | 39 |
| F-B-3 | B-3 | 100 | 51 | 37 |
| F-B-4 | B-4 | 100 | 50 | 36 |
| F-B-5 | B-5 | 100 | 64 | 50 |
| F-B-6 | B-6 | 100 | 69 | 55 |
| F-B-7 | B-7 | 100 | 53 | 39 |
| F-C-1 | - | - | 14 | - |

### <Production of test cigarette>

The commercially available filter-tipped cigarettes "Seven Stars Solid Menthol" were used for the preparation of test cigarettes. The filter of the commercially available cigarettes was removed. The resultant cigarette rod was connected to each of the filters (F-A-1, F-B-1 to F-B-7, and F-C-1) to produce test cigarettes. In this regard, the filter ventilation was set to 0. The cigarette prepared by using the filter F-C-1 is a control cigarette.

### <Smoking test>

The produced cigarettes were subjected to the smoking test according to the same procedure as Example 1. The sample for analysis obtained in the smoking test was used to analyze tar, nicotine, and the semivolatile components according to the same procedure as Example 1. The permeability (%) and the selective filtration coefficient (%) were calculated according to the same numerical formulae described in Example 1.

The permeability and selective filtration coefficient of the typical semivolatile components of the cigarettes obtained by using the filters F-A-1 and F-B-1 to F-B-7 are shown in Table 14 below.

### [Table 14]

**Table 14: Permeability and selective filtration coefficient of typical semivolatile components**

| Filter | F-A-1 | F-B-1 | F-B-2 | F-B-3 | F-B-4 | F-B-5 | F-B-6 | F-B-7 |
|---|---|---|---|---|---|---|---|---|
| Permeability (%) | 68 | 67 | 73 | 72 | 74 | 69 | 68 | 72 |
| Selective permeation coefficient (%) | 98 | 105 | 98 | 100 | 101 | 100 | 98 | 99 |

The permeability of the typical semivolatile components of the cigarettes obtained by using the filters F-A-1 and F-B-1 to F-B-7 is shown in FIG. 10.

From the results of Table 14 and FIG. 10, it can be confirmed that the permeability of the semivolatile components by the filtration rate control particles contained in each filter is constant regardless of the presence or absence of the additive or the kind of the additive. From this result, the following could be confirmed. Even if the additive contributing to cigarette smoking flavor is added to the filtration rate control particles, a small amount thereof does not have any influence on the filtering characteristics of the filtration rate control particles.

### List of Reference Signs

10 ... cigarette, 110 ... cigarette rod, 111 ... cigarette paper, 112 ... tobacco filler, 120 ... filter, 121 ... filter plug, 122 ... cellulose acetate fiber tow, 123 ... cellulose acetate fiber, 124 ... filtration rate control particles, 125 ... filter wrapping paper, 130 ... tipping paper, 131 ... ventilation hole, 140 ... acetate plain filter plug, 141 ... filter wrapping paper, 142 ... cellulose acetate fiber tow

## Claims

1. A cigarette filter comprising a filter plug that includes a filter material containing:
a cellulose acetate fiber tow, and
cellulose triacetate particles dispersed in the tow and having an average acetyl substitution degree of 2.8 to 3.0, wherein the cellulose triacetate particles do not contain any additives and have a BET specific surface area of less than 5 m²/g, and account for 1.5 to 30% by volume of the total volume of the filter plug.

2. The cigarette filter according to claim 1, **characterized in that** the cellulose triacetate particles account for 1.5 to 16% by volume of the total volume of the filter plug.

3. The cigarette filter according to any one of claims 1 or 2, **characterized in that** the cellulose triacetate particles have a sphere equivalent diameter of 100 µm to 1000 µm.

4. The cigarette filter according to any one of claims 1 to 3, **characterized in that** a plasticizer is added to the cellulose acetate fiber tow in an amount of 3% by weight or less based on the cellulose acetate fiber tow, or not added.

5. A filter-tipped cigarette comprising:
a cigarette rod; and
the cigarette filter according to any one of claims 1 to 4 which is attached to the end of the cigarette rod.

## Patentansprüche

1. Zigarettenfilter, der einen Filterstopfen umfasst, der ein Filtermaterial enthält, das Folgendes enthält:
ein Celluloseacetatfaserwerg und
Cellulosetriacetatpartikel, die in dem Werg dispergiert sind und einen durchschnittlichen Acetysubstitutionsgrad von 2,8 bis 3,0 aufweisen, wobei die Cellulosetriacetatpartikel keine Additive enthalten und einen spezifischen BET-Oberflächenbereich von weniger als 5 m²/g aufweisen und 1,5 bis 30 Volumen-% des Gesamtvolumens des Filterstopfens ausmachen.

2. Zigarettenfilter nach Anspruch 1, **dadurch gekennzeichnet, dass** die Cellulosetriacetatpartikel 1,5 bis 16 Volumen-% des Gesamtvolumens des Filterstopfens ausmachen.

3. Zigarettenfilter nach einem der Ansprüche 1 oder 2, **dadurch gekennzeichnet, dass** die Cellulosetriacetatpartikel einen Kugeläquivalenzdurchmesser von 100 µm bis 1.000 µm aufweisen.

4. Zigarettenfilter nach einem der Ansprüche 1 bis 3, **dadurch gekennzeichnet, dass** dem Celluloseacetatfaserwerg ein Weichmacher in einer Menge von 3 Gew.-% oder weniger, basierend auf dem Celluloseacetatfaserwerg, hinzugefügt wird oder nicht hinzugefügt wird.

5. Zigarette mit Filterspitze, umfassend:
ein Zigarettenstäbchen; und
den Zigarettenfilter nach einem der Ansprüche 1 bis 4, der am Ende des Zigarettenstäbchens befestigt ist.

## Revendications

1. Filtre de cigarette comprenant un bout filtre qui comprend un matériau de filtre contenant :
une filasse de fibre d'acétate de cellulose, et
des particules de triacétate de cellulose dispersées dans la filasse et ayant un degré moyen de substitution acétyle de 2,8 à 3,0, dans lequel les particules de triacétate de cellulose ne contiennent pas d'additif et présentent une surface spécifique BET inférieure à 5 m²/g, et comptent pour de 1,5 à 30 % en volume du volume total du bout filtre.

2. Filtre de cigarette selon la revendication 1, **caractérisé en ce que** les particules de triacétate de cellulose comptent pour de 1,5 à 16 % en volume du volume total du bout filtre.

3. Filtre de cigarette selon l'une quelconque des revendications 1 ou 2, **caractérisé en ce que** les particules de triacétate de cellulose présentent un diamètre équivalent de sphère de 100 µm à 1 000 µm.

4. Filtre de cigarette selon l'une quelconque des revendications 1 à 3, **caractérisé en ce qu'**un plastifiant est ajouté à la filasse de fibre d'acétate de cellulose dans une quantité de 3 % en masse ou inférieure sur la base de la filasse de fibre d'acétate de cellulose, ou n'est pas ajouté.

5. Cigarette à bout filtre comprenant :
une tige de cigarette ; et
le filtre de cigarette selon l'une quelconque des revendications 1 à 4 qui est fixé à l'extrémité de la tige de cigarette.
